



US006296923B1

(12) **United States Patent**  
**Zobel**

(10) **Patent No.:** **US 6,296,923 B1**  
(b4) **Date of Patent:** **Oct. 2, 2001**

(54) **PERFORATED POLYMERIC FILM WITH LIMITED OXYGEN AND WATER PERMEABILITY**

(75) Inventor: **Michael George Reinhardt Zobel**, Bridgwater (GB)

(73) Assignee: **Sidlaw Flexible Packaging Limited**, London (GB)

(\*) Notice: Subject to any disclaimer, the term of this patent is extended or adjusted under 35 U.S.C. 154(b) by 0 days.

(21) Appl. No.: **08/257,431**

(22) Filed: **Jun. 8, 1994**

**Related U.S. Application Data**

(63) Continuation of application No. 07/910,561, filed on Jul. 8, 1992, now abandoned, which is a continuation of application No. 07/629,621, filed on Dec. 18, 1990, now abandoned, which is a continuation of application No. 07/377,082, filed on Jul. 10, 1989, now abandoned.

(30) **Foreign Application Priority Data**

Jul. 15, 1988 (GB) ..... 8816950

(51) **Int. Cl.<sup>7</sup>** ..... **B65B 55/00**

(52) **U.S. Cl.** ..... **428/137; 428/131; 428/220; 428/315.5; 428/536; 428/516; 428/347; 428/338; 428/339; 428/523; 428/913; 426/415; 426/419; 426/326; 426/316; 426/410; 426/118; 426/395; 53/396; 53/141; 53/432; 53/469; 53/449**

(58) **Field of Search** ..... **428/131, 220, 428/315.5, 536, 516, 137, 347, 338, 339, 523, 913; 426/415, 419, 326, 316, 410, 118, 395; 383/102, 103; 53/396, 141, 432, 469, 449**

(56) **References Cited**

**U.S. PATENT DOCUMENTS**

|           |   |         |             |       |         |
|-----------|---|---------|-------------|-------|---------|
| 3,085,608 | * | 4/1963  | Mathues     | ..... | 383/103 |
| 3,224,898 |   | 12/1965 | Spencer     | ..... | 117/76  |
| 3,264,167 |   | 8/1966  | Sands       | ..... | 161/111 |
| 3,271,560 |   | 9/1966  | Schott, Jr. | ..... | 219/243 |
| 3,334,803 |   | 8/1967  | Abbey       | ..... | 229/53  |
| 3,471,597 | * | 10/1969 | Schirmer    | ..... | 264/25  |

|           |         |         |                   |         |          |
|-----------|---------|---------|-------------------|---------|----------|
| 3,546,327 | 12/1970 | Ruda    | .....             | 264/156 |          |
| 3,795,749 | *       | 3/1974  | Cummin et al.     | .....   | 426/326  |
| 3,880,966 | *       | 4/1975  | Zimmerman et al.  | .....   | 264/25   |
| 4,657,610 |         | 4/1987  | Komatsu et al.    | .....   | 156/87   |
| 4,735,843 |         | 4/1988  | Noda              | .....   | 428/137  |
| 4,876,146 | *       | 10/1989 | Isaka et al.      | .....   | 428/347  |
| 4,886,372 | *       | 12/1989 | Greengrass et al. | .....   | 383/100  |
| 4,897,274 | *       | 1/1990  | Candida et al.    | .....   | 426/127  |
| 4,935,271 | *       | 6/1990  | Schirmer          | .....   | 428/35.2 |

**FOREIGN PATENT DOCUMENTS**

|            |   |         |         |       |            |
|------------|---|---------|---------|-------|------------|
| 0039115    | * | 11/1981 | (EP)    | .     |            |
| 0155035    | * | 9/1985  | (EP)    | .     |            |
| 0270764    | * | 6/1988  | (EP)    | .     |            |
| 1106265    | * | 3/1968  | (GB)    | .     |            |
| 1134667    | * | 11/1968 | (GB)    | .     |            |
| 2068991    | * | 12/1980 | (GB)    | .     |            |
| 2179025    | * | 2/1987  | (GB)    | .     |            |
| 53-51096   |   | 5/1978  | (JP)    | ..... | B32B/7/02  |
| 54-40793   |   | 3/1979  | (JP)    | ..... | B65D/85/52 |
| 148247     | * | 7/1987  | (JP)    | .     |            |
| 62-235086/ |   |         |         |       |            |
|            |   | 1987    | 10/1987 | (JP)  | .          |

**OTHER PUBLICATIONS**

Briones et al., International Journal of Food Science and Technology (1992), 27, 493-505.

\* cited by examiner

Primary Examiner—William P. Watkins, III

(74) Attorney, Agent, or Firm—Bacon & Thomas, PLLC

(57) **ABSTRACT**

The invention provides polymeric films for the storage or packing of plant material, the film being perforate and having a water vapor permeability of not more than 800 g  $m^{-2}$  day $^{-1}$  and an oxygen permeability of not more than 200000  $cm^3 m^{-2}$  day $^{-1}$  atmosphere $^{-1}$ , both permeabilities being measured at 25° C. with a relative humidity of 75 percent. Examples of polymers which can be used to make the film are regenerated cellulose, homo and copolymers of polyolefins, e.g. with vinyl acetate or methyl acrylate, polyesters and polyamides. Various plant materials, for example carrots, tomatoes, calabrese and mushrooms heat sealed in packs of films of the invention have shown improved shelf lives compared with similar plant materials packaged for example in polyethylene cling film or polyvinyl chloride stretch wrap.

**19 Claims, No Drawings**

**PERFORATED POLYMERIC FILM WITH  
LIMITED OXYGEN AND WATER  
PERMEABILITY**

This application is a Continuation of application Ser. No. 07/910,561, filed Jul. 8, 1992, now abandoned, which is a Continuation of application Ser. No. 07/629,621, filed Dec. 18, 1990, now abandoned, which is a Continuation of application Ser. No. 07/377,082, filed Jul. 10, 1989, now abandoned.

**BACKGROUND OF THE INVENTION**

1. Field of the Invention

This invention concerns polymeric films, and in particular polymeric films for the storage or packaging of plant materials.

2. Description of the Prior Art

During storage, plant materials continue to respire even when the materials have been removed from the plant on which they were growing or when the plant material has been dug out of the ground. Thus fruit and vegetables, for example, continue to place demands on the surrounding atmosphere during storage, and deterioration of the quality of the plant materials occurs through water loss and surrounding levels of oxygen and carbon dioxide which do not favour their remaining fresh.

The freshness of fruit and vegetables can be prolonged by packaging, and this can have the added advantage of reducing damage when the fresh produce is displayed on a supermarket shelf. However, there are problems with the use of many packaging materials as the atmosphere within the package changes as respiration proceeds. This can be a particular problem with plant materials which undergo a climacteric stage during ripening, when a sharp rise in the rate of respiration occurs. Thus, while polymeric films, e.g. polyolefin films, can improve the shelf life of fruit and vegetables, a point can come during their storage when deterioration is accelerated by the changes in the atmosphere within the package.

Various proposals have been made for overcoming the problems with storing plant materials in packages made from polymeric films. British Patent Specifications 1106265 and 1134667, for example, describe control of the atmosphere within a package so that the oxygen content is less than that of normal air while the carbon dioxide content is greater than that of normal air, this being effected by the use of imperforate polyethylene sheet of a thickness that it is permeable to oxygen and carbon dioxide and of an area sufficient to allow the sealed-in produce to establish and maintain a controlled atmosphere within the package. Although oxygen and carbon dioxide levels are controlled by this method, the water content of the atmosphere is not and this can lead to undesirable water levels which can increase deterioration of the packaged materials.

Films with very high water permeability are proposed in Japanese Patent Publication 62.148247, 50 to 300 holes per square centimetre being made in the film, each hole being from 50 to 300 microns in diameter. These films are proposed for wrapping cut flowers where the water vapour permeability has to be sufficient to remove condensed water droplets.

Other proposals include the use of as and water-vapour impermeable films which have permeable windows let into them, the windows being made of more permeable materials. Alternatively, composite containers have been proposed

in which one side of the container is made from an impermeable plastics film and another side is made from a microporous film.

**SUMMARY OF THE INVENTION**

According to the present invention there is provided a polymeric film for the storage or packaging of plant material, the film being perforate and having a water vapour permeability of not more than  $800 \text{ g m}^{-2} \text{ day}^{-1}$  and an oxygen permeability of not more than  $200000 \text{ cm}^3 \text{ m}^{-2} \text{ day}^{-1} \text{ atmosphere}^{-1}$ , both permeabilities being measured at  $25^\circ \text{ C}$ . with a relative humidity of 75 percent.

**DETAILED DESCRIPTION OF THE  
PREFERRED EMBODIMENTS**

Films of the present invention have the advantage of providing packages with the desired degree of oxygen permeability to give good storage life to plant materials stored in them while at the same time enabling the water permeability of the packages to be controlled to a desired level, this being achieved without the necessity for special windows or a number of films for the one package. Films of the present invention can be produced which are generally stiffer than conventional cling film, thus enabling them to be used more readily on horizontal or vertical form fill seal packaging machinery. Furthermore, they will usually be clear as the perforations used are very small.

The water vapour permeability of the films of the present invention can be selected by the type of polymer used for the film. Examples of polymers which can be used include regenerated cellulose, homo and copolymers of polyolefins, e.g. with vinyl acetate or methyl acrylate, polyesters and polyamides. The films can furthermore be laminates and/or can include one or more layers, e.g. a heat sealable layer. Films of regenerated cellulose can be used to achieve water vapour permeability over a wide range, typically up to  $800 \text{ g m}^{-2} \text{ day}^{-1}$  measured at  $25^\circ \text{ C}$ . and 75 percent relative humidity for a film 24 microns thick. Lower permeabilities can be achieved by the use of a thicker film, but it is generally preferred to apply a coating to the film when it is desired to reduce its permeability to water vapour. Suitable materials for the purpose are known in the art. Thus water vapour permeabilities of  $100$ – $800 \text{ g m}^{-2} \text{ day}^{-1}$  can be achieved, and if desired lower values, e.g. down to  $80 \text{ g m}^{-2} \text{ day}^{-1}$ , or even lower, e.g. as little as  $10 \text{ g m}^{-2} \text{ day}^{-1}$  can be achieved. When a coating is present, the permeability will usually be less than  $500 \text{ g m}^{-2} \text{ day}^{-1}$ .

Polyolefins can also be used to make films of the present invention, the inherent water vapour permeability of films of such materials tending to be substantially less than that of uncoated regenerated cellulose films of the same thickness. Polyethylene films 30 microns thick typically have water vapour permeabilities of about  $4 \text{ g m}^{-2} \text{ day}^{-1}$ , while polypropylene films of the same thickness typically have water vapour permeabilities of  $1$ – $2 \text{ g m}^{-2} \text{ day}^{-1}$ .

The water vapour permeability of the film will be selected to suit the respiration requirements of the plant material to be packaged, and therefore there are no overall preferences for water vapour permeability other than that the permeability be selected to optimise the storage life of the packaged plant material.

The oxygen permeability of films of the present invention is not more than  $200000 \text{ cm}^3 \text{ m}^{-2} \text{ day}^{-1} \text{ atmosphere}^{-1}$  as measured at  $25^\circ \text{ C}$ . and 75 percent relative humidity. As with water vapour permeability, different plant materials require films with different oxygen permeabilities, and permeability

ties of not more than 100000, e.g. less than  $50000 \text{ cm}^3 \text{ m}^{-2} \text{ day}^{-1}$  atmosphere $^{-1}$  are often preferred. Lower oxygen permeabilities still can be achieved, for example less than  $10000 \text{ cm}^3 \text{ m}^{-2} \text{ day}^{-1}$  atmosphere $^{-1}$ . The oxygen permeability will, however, be greater than that inherent for the material of the film, and typically it should be at least  $900 \text{ cm}^3 \text{ m}^{-2} \text{ day}^{-1}$  atmosphere $^{-1}$  greater than that of the material of the film. This usually means at least  $3500 \text{ cm}^3 \text{ m}^{-2} \text{ day}^{-1}$  atmosphere $^{-1}$ .

The oxygen permeability of films of the present invention is achieved by perforations in the film. The size of the perforations affects the oxygen permeability of the film, and they are preferably from 20 to 100 microns, more preferably 40 to 60 microns and advantageously about 50 microns mean diameter. If the perforations are too large, control of oxygen permeability is not possible, and if the holes are too small, large numbers of holes are required which in particular adds to the cost of the film. Typically it is preferred to have up to 1000 perforations in the film per square metre of film surface, but as few as 10 perforations or even less can be used. These sizes (20 to 100 microns, preferably 40 to 60 microns) and numbers (100 to 1000 per  $\text{m}^2$  of film surface) represent a percentage of perforations in the range of  $3.14 \times 10^{-7}$  to  $7.85 \times 10^{-4}\%$ , preferably  $1.26 \times 10^{-6}$  to  $2.83 \times 10^{-4}\%$  of the total film surface. This is very significantly lower than the frequency of perforations in the films proposed in Japanese Patent Publication 62.148247 which proposes 50 to 300 holes per square centimeter, i.e. at least five hundred times fewer perforations for the same area of film. As will be appreciated, the size and number of perforations in films in accordance with the invention will be selected according to the plant material to be packaged. However, there should be sufficient perforations in the film that each package of plant material has at least one perforation. This usually requires at least 50 perforations per square meter. Usually the film will have fewer than 500 perforations per square meter, and typically from 100 to 300 per square meter.

The holes or perforations in films of the present invention can be produced by known methods. It is, however, unlikely that they will be sufficiently small to achieve the desired oxygen permeability if mechanical puncturing methods are used, and the preferred methods are electrical discharge and optical means, e.g. using a laser.

In most applications, it will be necessary to be able to heat seal films of the present invention, in particular to ensure that the oxygen permeability depends on the perforations in the film rather than leaks in the package. Various heat sealable layers can therefore be present on films of the present invention, and as will be appreciated these will affect the inherent water vapour permeability of the films. Of course, the film itself may be of a heat sealable material.

As will be appreciated by those skilled in the art, any heat sealable layer or other layer should not obscure the perforations in the film, and the perforations will therefore usually be made in a film already having such layers. These layers, which can be selected from those known in the art, can be formed in known manner, for example by co-extrusion or by coating.

In packaging plant materials, the film will be selected to meet the requirements of the material to be packaged, both in terms of water vapour permeability (i.e. the type and thickness of polymer used for the film) and oxygen permeability (i.e. the size and frequency of perforations, these also differing for the same material under different temperature conditions.) Obviously when very small numbers of perforations are used, e.g. about 10 per square meter, the amount

of film used for an individual pack should be such as to include at least one perforation in the surface of the film so that oxygen can pass between the interior of the pack and the atmosphere outside.

Various types of fruits, vegetables, herbs and flowers have shown particularly good shelf lives when stored in packages made from films of the present invention. Thus broccoli, carrots, mushrooms and tomatoes, which represent a wide variety of plant materials in terms of requirements for oxygen, carbon dioxide and water vapour during respiration, have all shown extended shelf lives when compared with those packed in hitherto proposed polymeric packaging films.

The following Examples are given by way of illustration only. All parts are by weight and all temperatures are in °C. unless stated otherwise.

#### EXAMPLE 1

After discarding any showing signs of damage, carrots were washed, placed for 1 minute in chilled water containing 25 ppm of chlorine, and then rinsed with cold water. The carrots were allowed to dry, and packs were prepared by heat sealing them in a variety of films, each pack having internal dimensions of 20 cm x 18 cm and containing approximately 0.35 kg of carrots. A similar quantity of carrots on an open tray without any wrapping film acted as a control. The samples were all stored at 20° C. and 50 percent relative humidity.

The films used were as follows:

- (A)—heat sealable oriented polypropylene 25 microns thick and having 100 holes per square meter, the mean diameter of the holes being about 50 microns
- (B)—as film (A) but with 68 holes per square meter
- (C)—as film (A) but with 34 holes per square meter
- (D)—as film (A) but without any holes
- (E)—imperforate polyethylene cling film 25 microns thick
- (F)—imperforate polyvinyl chloride stretch wrap film 25 microns thick

All of the packs having a film over the carrots had a much improved shelf life compared with the unwrapped control. The packs had mould free shelf lives of at least seven days, the unwrapped carrots becoming dried, shrivelled and unacceptable after three days. The packs wrapped with the imperforate films (D), (E) and (F) either became anaerobic within three days or were becoming so by 10 days. The carrots wrapped in film (B) were particularly good, those wrapped in films (A) and (C) being somewhat less so but still significantly better than those wrapped in the other films.

Water losses from all of the packaged carrots were acceptable in all cases at less than 1% by weight after 10 days.

#### EXAMPLE 2

The procedure of Example 1 was repeated for tomatoes except that they were packed in trays of six after washing and then drying for one hour. The calices were not removed.

Each tray was wrapped in one of the films (A) and (C)–(F) of Example 1, and a further tray was left unwrapped as a control.

The unwrapped tomatoes became very soft and mouldy after four days, and those wrapped in film (F) became mouldy after three days. Film (A), with 100 holes per square meter, led to widespread mould after seven days, the toma-

toes having become soft after four days. However, tomatoes packed in film (C) remained firm even after six days.

## EXAMPLE 3

Packs of unwashed calabrese were prepared by wrapping 150 g of the calabrese on trays 025 m $\times$ 0.185 m (area 0.0925 m $^2$ ), the films being:

(G)—25 micron thick heat sealable oriented polypropylene film

(H)—film (G) with 21 holes over pack area

(I)—film (G) with 7 holes over pack area

For comparison purposes, 150 g samples of calabrese were packed in 25 microns thick polyvinyl chloride cling film or simply left unwrapped.

The unwrapped pack was very limp and showed browning after two days at 20° C. and 50 percent relative humidity. Under the same conditions, the calabrese packed in the polyvinyl chloride cling film showed yellowing after two days whereas the perforated films of the present invention did not show adverse signs until nearly six days. After three days, the calabrese packed in the unperforated polypropylene film showed dry ends and it was limper than that in the perforated film. At 4° C., calabrese stored in films of the present invention were still very good and fresh after 17 days and of better appearance than any of the samples packed using the other films.

## EXAMPLE 4

Using the procedure of Example 3, 200 g of unwashed mushrooms were packed in a variety of films as follows:

(J)—unperforated heat sealable regenerated cellulose film 25 microns thick and having a water vapour permeability of 80 g m $^{-2}$  day $^{-1}$ —pack size 0.25 m $\times$ 0.185 m (area 0.0925 m $^2$ )

(K)—film (J) with 53 holes over pack area—pack size 0.175 m $\times$ 0.125 m (area 0.0875 m $^2$ )

(L)—as film (K) but with 25 holes over same pack area

(M)—as film (K) but with 12 holes over same pack area

Comparison tests were also carried out using 25 micron thick polyvinyl chloride cling film with 200 g of mushrooms on a 0.175 m $\times$ 0.125 m tray and with the same amount of mushrooms unwrapped, the packs being stored at 20° C. and 50 percent relative humidity.

The unwrapped mushrooms were unacceptable after two days, as were those packed in the cling film and in film (J). The mushrooms packed in film (K) were still acceptable approaching six days, whereas those packed in films (L) and (M) were showing significant signs of deterioration after three days.

A similar series of tests at 4° C. using films of the present invention based on the same regenerated cellulose film but with 12, 25 and 50 holes respectively over the pack area showed very good results at up to 20 days whereas the

unperforated film and the cling film led to an unacceptable product and in some cases mould formation after only two days.

What is claimed is:

- 5 1. A polymeric film for the storage or packaging of plant material, the film having from 10 to 1000 perforations per square meter therein, wherein the mean diameter of the perforations is from 20 to 100 microns, said film having a water vapour permeability of not more than 800 g m $^{-2}$  day $^{-1}$  and an oxygen permeability of not more than 200000 cm $^3$  m $^{-2}$  day $^{-1}$  atmosphere $^{-1}$ , both permeabilities being measured at 25° C. with a relative humidity of 75 percent.
- 10 2. A film according to claim 1, wherein the film is of regenerated cellulose.
- 15 3. A film according to claim 2, wherein the regenerated cellulose has a coating thereon which modifies the water vapour permeability of the film.
- 20 4. A film according to claim 1, wherein the water vapour permeability is from 100 to 800 g m $^{-2}$  day $^{-1}$ .
- 25 5. A film according to claim 1, wherein the water vapour permeability is at least 10 g m $^{-2}$  day $^{-1}$ .
- 30 6. A film according to claim 1, wherein the film is of a polyolefin.
- 35 7. A film according to claim 6, wherein the polyolefin is polyethylene or polypropylene.
- 40 8. A film according to claim 1, wherein the oxygen permeability of the film is not more than 100000 cm $^3$  m $^{-2}$  day $^{-1}$  atmosphere $^{-1}$ .
- 45 9. A film according to claim 8, wherein the oxygen permeability of the film is less than 50000 cm $^3$  m $^{-2}$  day $^{-1}$  atmosphere $^{-1}$ .
- 50 10. A film according to claim 9, wherein the oxygen permeability is less than 10000 cm $^3$  m $^{-2}$  day $^{-1}$  atmosphere $^{-1}$ .
- 55 11. A film according to claim 1, wherein the mean diameter of the perforations is from 40 to 60 microns.
- 60 12. A film according to claim 11, wherein the mean diameter of the perforations is about 50 microns.
- 65 13. A film according to claim 1, which is clear.
- 70 14. A film according to claim 1, having at least one heat sealable surface.
- 75 15. A film according to claim 1, having perforations therein representing from 1.26 $\times$ 10 $^{-6}$  to 2.83 $\times$ 10 $^{-4}$  percent of the film surface area.
- 80 16. A film according to claim 1, wherein the water vapour permeability is at least 80 g m $^{-2}$  day $^{-1}$ .
- 85 17. A respiring plant material packaged in the polymeric film of claim 1.
- 90 18. The packaged respiring plant material of claim 17 wherein the respiring plant material is a fruit or vegetable.
- 95 19. The packaged material according to claim 18 wherein the fruit or vegetable is broccoli, carrots, mushrooms or tomatoes.

\* \* \* \* \*